

# UNITED STATES PATENT OFFICE.

HILYARD STOKES, OF BEVERLY, NEW JERSEY, ASSIGNOR OF ONE-THIRD TO JONATHAN E. WRIGHT, OF PHILADELPHIA, PENNSYLVANIA, AND ONE-THIRD TO MITCHELL B. PERKINS, OF BEVERLY, NEW JERSEY.

## WOOD-PRESERVING COMPOSITION.

No. 896,835.

Specification of Letters Patent. Patented Aug. 18, 1908.

Application filed February 17, 1908. Serial No. 416,384.

To all whom it may concern:

Be it known that I, HILYARD STOKES, a citizen of the United States, and a resident of Beverly, Burlington county, New Jersey, have invented certain Improvements in Wood Preservatives and in the Mixing of the Same, of which the following is a specification.

My invention relates to compositions of matter employed for the preservation of wood and other fibrous material of a similar nature, such as are applied by coating the wood or other material externally, or by soaking the same to secure a high degree of saturation or penetration, a condition that will be accentuated by heat as well as by the porosity of the material treated.

The object of my invention is to provide a material that will not only kill any insect life or larvæ present in the wood or other fibrous material, but will also afford such a coating and impregnation as to resist moisture and its deleterious effects; the attack of insects or marine animals, and all conditions that would tend to cause decay or other deterioration.

The improved compound forming the subject of my invention is composed of an excess of crude mineral oil, with which is associated animal fat such as lard, grease collected from animal refuse in the manufacture of fertilizers, tallow, or wool oil, together with oil from certain marine animals, and a salt of an alkaline carbonate, such as sal soda ( $Na_2CO_3 \cdot 10H_2O$ ). Of the materials so named, I prefer to use crude petroleum, lard, fish oil, and sal soda, and in making my improved preservative, I use these ingredients mixed or combined in substantially the following proportions:

|                                      |           |
|--------------------------------------|-----------|
| Mineral oil (crude petroleum)        | 74. parts |
| Lard (melted)                        | 14.8 "    |
| Fish oil                             | 7.4 "     |
| Sal soda ( $Na_2CO_3 \cdot 10H_2O$ ) | 3.8. "    |

These ingredients or their equivalents are incorporated in the presence of heat by first heating the fish oil to 100° F., then adding the pulverized sal soda, stirring this mixture until sal soda becomes entirely dissolved, then add and mix well the melted animal fat, finally adding the petroleum slowly and stirring so as to get a perfect mixture, keeping the entire solution warm for at least two or

three hours to procure a homogeneous condition.

The main ingredient, crude oil, together with the lard and fish oil, or their equivalent form the body of the composition, and the sal soda or its equivalent is added to keep the mixture pliable, being combined therewith, so that when applied to wood it will prevent that portion remaining on the surface from checking or cracking, as well as on account of its penetrating properties, which it imparts to the whole composition, enabling it to much more readily and perfectly fill the pores and fibers of the wood.

My improved preservative may be made in any suitable receptacle and preferably in the vessel in which the wood or other material is to be treated; such receptacle or vessel being so arranged as to be susceptible of being heated to the degree necessary for a homogeneous combination of the several elements forming such composition.

In naming the proportions which may be employed, I do not wish to be limited to the exact figures given, as quantities may vary depending upon the specific use to which the compound is to be put and character of the material treated, as the ultimate desire is to coat or impregnate such wood to such an extent that any cracks or porous spots not apparent to the eye shall be thoroughly saturated or covered as to prevent absolutely the reception and retention of moisture; to kill all insects and larvæ present; to resist the attack of insects or marine animals, and to prevent decay incident to continued exposure to the elements or due to contact with the ground.

An important point in connection with my improved material is the method of applying the same for the preservation of wood. Primarily speaking, it has been designed particularly for the purpose of treating railroad ties, although it can be used for treating wood employed for any purpose or where it is subject to the elements, the ravages of insect life or marine animals, or to dampness incident to its position in the ground. In treating such wood, railroad ties and the like, I prepare a bath; this bath to contain the ingredients noted, incorporated in the manner described, that is to say, to have a temperature substantially at or about 200° F.; while it may be desirable to boil or nearly

boil the ingredients in effecting the thorough incorporation of the same, it is not absolutely necessary to have the preservative in this condition when treating the wood and other material.

5 The wood should preferably be well seasoned and substantially dry, having had its normal water contents dispelled by the aid of heat. It will be understood, of course, that the drier the wood, the easier the penetration of the preservative. Such wood is then placed in the heated bath and allowed to remain there for a period of about three hours.

10 15 After the wood is removed from the bath it is permitted to dry, the preservative having soaked into the wood, so that the latter presents substantially its original appearance. Should the preservative effect an undesirable discoloration of the wood, coloring matter may be added to the preservative to offset such condition. This treatment of wood, when applied to railroad ties, has the effect of increasing the normal holding 20 25 power of spikes after being driven. I believe that it will prevent the spikes from working up or out of the ties.

To sawed timber, presenting a relatively smooth surface, the preservative may be applied in the hot condition with a brush; repeated applications of the same being given thereto instead of soaking such wood in a receptacle, such for instance as that in which

the solutions are mixed. This arrangement may be particularly desirable in cases where 35 the material to be treated is of such a size as to prevent it soaking in the tank, or where it is desired to apply the preservative to a building under construction, or one already built. Under ordinary circumstances, however, I prefer to saturate the wood to be treated in the manner described. Piles for marine work may be treated with this preservative, and it is well adapted for coating shingles.

40 45 I claim:

1. The herein described composition of matter for the preservation of wood and other fibrous material consisting of a mixture of a soda soap derived from fish oil and lard and combined with crude mineral oil in excess.

2. The herein described composition of matter for the preservation of wood and other fibrous materials, consisting of a mixture of a soda soap derived from fish oil 7.4 parts, lard 14.8 parts and sal soda 3.8 parts, combined with 74 parts by volume of crude mineral oil.

55 In testimony whereof, I have signed my name to this specification, in the presence of two subscribing witnesses.

60 HILYARD STOKES.

Witnesses:

MURRAY C. BOYER,  
JOS. H. KLEIN.